# EUROPEAN PATENT SPECIFICATION

(11) **EP 0 059 023 B1**
(45) Date of publication and mention of the grant of the patent: **30.04.1986**
(21) Application number: 82300025.2
(22) Date of filing: 05.01.1982
(51) Int. Cl.: C23D 3/00

(54) **Process for improving the corrosion resistance of a ferrous metal body**
Verfahren zur Verbesserung der Korrosionsbeständigkeit eiserner Gegenstände
Procédé pour améliorer la résistance à la corrosion d'un article en métal ferreux

(30) Priority: 16.01.1981 GB 8101306
(43) Date of publication of application: 01.09.1982
(73) Proprietor: International Standard Electric Corporation, New York New York 10022 (US)
(72) Inventor: Drake, Cyril Francis, Harlow Essex (GB)
(74) Representative: Dennis, Mark Charles

## Description

This invention relates to corrosion inhibition and in particular to the prevention or inhibition of the corrosion of ferrous metals. The invention also relates to ferrous metal piece parts provided with such corrosion protection.

Ferrous metals are employed in the construction of reinforcing member in a variety of building and constructional operations. Typically the metal is used in the form of rods or wires which are embedded in concrete to form a structure having both tensile and compressive strength. Such reinforced concrete structures are employed e.g. in the construction of roadways, bridges, tunnels and buildings. In applications where a high load is to be applied to the reinforced structure it is often prestressed by applying tension to the reinforcing metal 'skeleton' thus enhancing the load bearing properties of the structure.

A problem associated with all ferrous metal structures is that of corrosion and consequent deterioration of the load bearing properties of the structure. This problem is particularly acute when the metal is in contact with or embedded in a building material such as cement or concrete. The commonly used building cements and concretes are strongly alkaline when freshly mixed with water and are highly corrosive in nature. A ferrous material is immediately attacked during the setting process and, as small traces of water remain in contact with the metal, this attack continues throughout the life of the composite structure. In some cases this can lead to the ultimate failure of the reinforcement.

Whereas composite structures of this type are used in low stress application this failure of the reinforcement can lead to fracture of the structure necessitating eventual replacement which can be difficult and costly. Where the composite structure is used in a high stress application sudden failure of one or more reinforcing members can lead to catastrophic failure with the partial or complete collapse of the structure.

Various techniques for preventing ferrous metal corrosion have been investigated. One of the best known techniques is that of dip coating the metal with a layer of zinc, the process being known as galvanizing. This process provides an effective degree of corrosion inhibition but, as the zinc coating is relatively thick, the process is too costly for many applications. Furthermore the period during which the corrosion inhibition is effective is limited in a corrosive environment by dissolution of the zinc which acts as a sacrificial anode. In an attempt to overcome the disadvantages of galvanised ferrous metal it has been proposed to protect the metal surface with a layer of electroplated copper which layer is chemically inert in many corrosive environments. However it has been found necessary to employ a relatively thick and therefore expensive, copper layer to avoid the risk of pinholes through which accelerated electrolytic corrosion of the ferrous metal can occur. Also abrasion damage to the copper layer exposes the underlying metal and again leads to electrolytic corrosion.

A further technique is disclosed in French specification No. 2,225,545. This describes a process for enamelling an iron or steel surface wherein, prior to application and firing of the enamel, the ferrous metal is provided with a protective surface layer of copper. This prevents corrosion of the ferrous metal beneath the enamel but suffers from the disadvantage that pinholing of the enamel can lead to rapid electrolytic corrosion.

The object of the invention is to minimise or to overcome these disadvantages.

According to the invention there is provided a ferrous metal body having a corrosion inhibiting surface coating, said coating including a layer of copper in contact with the metal surface and an external layer wholly or partially comprising a material having corrosion inhibiting properties, characterised in that said corrosion inhibiting material comprises a water soluble phosphorus pentoxide/zinc oxide/alumina glass.

According to another aspect of the invention there is provided a method of inhibiting corrosion of a ferrous metal surface, including applying a coating of copper to the surface, and covering the copper with a corrosion inhibiting coating, characterised in that said coating wholly or partially comprises a water soluble phosphorus pentoxide/zinc oxide/alumina glass.

Preferably the corrosion inhibiting material comprises a water soluble glass.

Embodiments of the invention will now be described with reference to the accompanying drawings in which:-
Figure 1 is a schematic diagram of a plant for producing corrosion inhibited ferrous metals; and
Figure 2 is a cross-section of a ferrous metal body produced by the plant of Figure 1.

Referring to the drawings, the coating plant shown in Figure 1 is intended for the treatment of e.g. steel rod or wire, or wire products, in continuous lengths. It will however be clear to those skilled in the art that the process can be readily adjusted to the treatment of ferrous metals in other forms such as tube and sheet.

The wire or wire product 11 to be treated is fed from a storage reel 12 through an electroplating bath 13 where a flash coating 21 (Fig. 2) of copper is deposited on the metal surface. To effect this coating an electric current is fed to the wire product 11 via one or more brush contacts 14, the current being fed via the wire through the electrolytic solution in the bath 13 to a copper anode 15. The thickness of the electrodeposited copper coating 21 can be determined by controlling both the site at which the wire product is fed through the plating bath 13 and the electroplating current. Typically this thickness will be in the range 0.01 to 1 pm although the thickness of the copper layer is not critical.

After the electrodeposition stage .the wire 11 passes, preferably via a washing and drying station 16 where electrolyte residues are removed, to a coating station 17 where the copper coated wire is provided with an outer corrosion inhibiting coating 22 (Fig. 2) comprising wholly or partially a water soluble glass housing corrosion inhibiting properties. Typically the glass is of the phosphorus pentoxide type and comprises phosphorus pentoxide/zinc oxide/alumina glass, such glass being described in our published United Kingdom specification No. 1,604,383. Advantageously the glass is applied as a powder dispersed in a paint resin, but other coating techniques may also be employed. Thus, for example, the glass may be applied as a fine powder from a fluidized bed followed by fusion of the glass to provide a uniform surface layer. Other coating methods will be apparent to those skilled in the art. Finally the coated wire 11 is wound on to a storage reel 18.

The corrosion inhibited ferrous metal products manufactured by the plant of Figure 1 may be employed in a variety of applications in hostile environments where unprotected ferrous metals would be subject to rapid corrosion. Advantageously the corrosion inhibited metal product is in the form of rods or wires which are employed as the reinforcing elements in cement and concrete structures; the corrosion inhibiting glass prevents attack of the ferrous metal during the concrete setting process and continues this protection for an extended period while the structure is in service.

Other applications include the corrosion inhibition of steel tube that is to be employed in the construction of underground or submarine pipelines e.g. for gas or oil.

## Claims

1. A ferrous metal body having a corrosion inhibiting surface coating, said coating including a layer of copper in contact with the metal surface and an external layer wholly or partially comprising a material having corrosion inhibiting properties, characterised in that said corrosion inhibiting material comprises a water soluble phosphorus pentoxide/zinc oxide/alumina glass.

2. A metal body as claimed in claim 1, characterised in that the glass is in the form of a powder dispersed in a paint resin.

3. A metal body as claimed in claim 1 or 2, characterised in that said copper layer is an electrodeposited layer.

4. A metal body as claimed in any one of claims 1 to 3, characterised in that said copper layer is from 0.01 to 1 pm thick.

5. A metal body as claimed in any one of claims 1 to 4 and in the form of a wire or a wire product.

6. A cement or concrete structure reinforced with a wire or wire product as claimed in claim 5.

7. A method of inhibiting corrosion of a ferrous metal surface, including applying a coating of copper to the surface, and covering the copper with a corrosion inhibiting coating, characterised in that said coating wholly or partially comprises a water soluble phosphorus pentoxide/zinc oxide/ alumina glass.

8. A method as claimed in claim 7, characterised in that said copper coating is electrodeposited.

9. A method as claimed in claim 7 or 8, characterised in that the copper coating is from 0.01 to 1 pm thick.

10. A method as claimed in claim 7, 8 or 9, characterised in that said glass is applied in the form of a powder dispersed in a paint resin.

## Revendications

1. Corps en métal reffeux comportant un revêtement de surface inhibiteur de la corrosion, ledit revêtement comprenant une couche de cuivre en contact avec la surface du métal et une couche externe comportant, partiellement ou dans sa totalité, un matériau ayant des propriétés inhibitrices de la corrosion, caractérisé en ce que ledit matériau inhibiteur de la corrosion comporte un verre d'alumine/oxyde de zinc/et pentoxyde de phosphore soluble dans l'eau.

2. Corps en métal selon la revendication 1 caractérisé en ce que le verre est sous la forme d'une poudre dispersée dans une résine de peinture.

3. Corps en métal selon la revendication 1 ou 2 caractérisé en ce que ladite couche de cuivre est une couche déposée par électrodéposition.

4. Corps en métal selon l'une quelconque des revendications 1 à 3 caractérisé en ce que ladite couche de cuivre a une épaisseur comprise entre 0,01 et 1 pm.

5. Corps en métal selon l'une quelconque des revendications 1 à 4 sous la forme d'un fil ou d'un produit filé.

6. Structure en ciment ou en béton, renforcée avec du fil ou un produit filé selon la revendication 5.

7. Procédé pour inhiber la corrosion de la surface d'un métal ferreux qui consiste à appliquer une couche de cuivre sur la surface, et à recouvrir le cuivre avec un revêtement inhibiteur de la corrosion, caractérisé en ce que ledit revêtement comporte, partiellement ou dans sa totalité, un verre d'alumine/oxyde de zinc/et pentoxyde de phosphore soluble dans l'eau.

8. Procédé selon la revendication 7, caractérisé en ce que ladite couche de cuivre est déposée par électrodéposition.

9. Procédé selon la revendication 7 ou 8, caractérisé en ce que la couche de cuivre a une épaisseur comprise entre 0,01 et 1 pm.

10. Procédé selon l'une des revendications 7, 8 ou 9, caractérisé en ce que ledit verre est appliqué sous la forme d'une poudre dispersée dans une résine de peinture.

## Patentansprüche

1. Eisenmetallkörper mit einem Korrosionsschutzüberzug, der eine in Kontakt mit der Metalloberfläche befindliche Kupferschicht und eine ganz oder teilweise aus- einem Korrosionsinhibitor bestehende äußere Schicht aufweist, dadurch gekennzeichnet, daß der Korrosionsinhibitor ein wasserlösliches Phosphorpentoxid-Zinkoxid-Aluminiumoxid-Glas ist.

2. Metallkörper nach Anspruch 1, dadurch gekennzeichnet, daß das Glas in Form eines in einem Lackharz dispergierten Pulvers vorliegt.

3. Metallkörper nach Anspruch 1 oder 2, dadurch gekennzeichnet, daß die Kupferschicht eine galvanisch aufgebrachte Schicht ist.

4. Metallkörper nach einem der Ansprüche 1 bis 3, dadurch gekennzeichnet, daß die Dicke der Kupferschicht 0.01 bis 1 pm beträgt.

5. Metallkörper nach einem der Ansprüche 1 bis 4 und in Form eines Drahtes oder Drahtprodukts.

6. Zement- oder Betonkonstruktion, die mit einem Draht oder Drahtprodukt nach Anspruch 5 bewehrt ist.

7. Verfahren zum Schutz einer Eisenmetalloberfläche gegen Korrosion, bei dem eine Kupferschicht auf die Oberfläche aufgebracht wird und das Kupfer mit einem Korrosionsschutzüberzug versehen wird, dadurch gekennzeichnet, daß der Überzug ganz oder teilweise aus wasserlöslichem Phosphorpentoxid-Zinkoxid-Aluminiumoxid-Glas besteht.

8. Verfahren nach Anspruch 7, dadurch gekennzeichnet, daß die Kupferschicht galvanisch aufgebracht wird.

9. Verfahren nach Anspruch 7 oder 8, dadurch gekennzeichnet, daß die Dicke der Kupferschicht 0.01 bis 1 pm beträgt.

10. Verfahren nach Anspruch 7, 8 oder 9, dadurch gekennzeichnet, daß das Glas in Form eines in einem Lackharz dispergierten Pulvers aufgebracht wird.
